

# UNITED STATES PATENT OFFICE.

SAMUEL PEACOCK, OF PHILADELPHIA, PENNSYLVANIA, ASSIGNOR, BY MESNE ASSIGNMENTS, TO AGRICULTURAL RESEARCH CORPORATION, OF NEW YORK, N. Y., A CORPORATION OF NEW YORK.

## VOLATILE MAGNESIUM COMPOUNDS AND PROCESS OF PRODUCING SAME.

1,134,412.

Specification of Letters Patent.

Patented Apr. 6, 1915.

No Drawing.

Application filed April 18, 1914. Serial No. 832,810.

*To all whom it may concern:*

Be it known that I, SAMUEL PEACOCK, a citizen of the United States, residing at Philadelphia, in the county of Philadelphia and State of Pennsylvania, have invented 5 certain new and useful Improvements in Volatile Magnesium Compounds and Processes of Producing Same; and I do hereby declare the following to be a full, clear, and 10 exact description of the invention, such as will enable others skilled in the art to which it appertains to make and use the same.

This invention relates to a process of producing a volatile compound of carbon, nitrogen 15 and magnesium from an oxid of magnesium, gaseous nitrogen and carbon.

My invention also relates to the new volatile product produced by this process and has for its object the fixation of free nitrogen 20 in a manner more efficient and less expensive than the methods heretofore proposed.

With these and other objects in view the invention consists in the new product and 25 novel steps constituting my process more fully hereinafter disclosed and particularly pointed out in the claims.

In carrying out my process I prepare a charge of finely divided oxid of magnesium 30 and carbon, suitably proportion the same, and preferably briquet the said charge. I then introduce the charge into a suitable furnace. Gaseous nitrogen, or producer gas is introduced into the furnace chamber; and 35 an electric current is turned on, or other suitable heating means is employed, to raise the temperature to say substantially 1500° C., whereupon I have reason to believe the following reaction takes place:—



I have now discovered that the carbo-nitrid thus formed in the high temperature zone of the furnace is in a volatile as well as 45 in a solid form, and that the proportion of volatile to solid product depends in a measure upon the pressure existing in the furnace at the time of formation. In other words, I have discovered that when the furnace 50 pressure is above that of the atmosphere the proportion of volatile to solid carbo-nitrid produced is less than is the case when the pressure is that of the atmosphere; and that when the pressure is less than that of the

atmosphere the proportion of volatile product is greater than is the case when the atmospheric pressures exists in the furnace. For example when the pressure in the furnace is maintained for 30 minutes at 1000 m. m. of mercury, about 75% of the carbo-nitrid formed is volatilized while the remainder was found as a solid in the charge; when the pressure is maintained at 760 m. m. for the same period substantially all the carbo-nitrid is volatilized; and when the pressure is less than that of the atmosphere all the carbo-nitrid is volatilized in a period of time less than 30 minutes.

Either nitrogen gas or producer gas may be employed as above stated, and when producer gas is employed such gas may contain on the average about 60% nitrogen, N<sub>2</sub>, and 38% carbon monoxid, CO, so that when the nitrogen is removed by my process the producer gas is greatly improved and enriched 70 by the carbon monoxid CO, generated by the reaction. Therefore, said producer gas after coming from the furnace can later be utilized to a greater advantage for combustion or other purposes. That is to say, from 75 the carbo-nitrid equation, above, it is evident that for each volume of nitrogen fixed, an equal volume of carbon monoxid CO, is liberated, and joins the furnace gases. Now when producer gas is employed, having say 80 60% of nitrogen and 38% of carbon monoxid, and when one third or 20% of the nitrogen is fixed, it is evident that 20% of carbon monoxid will still be added to the 85 38% of carbon monoxid already present. Accordingly the resulting mixture will contain 58% of carbon monoxid instead of its 90 original 38%. It follows, therefore, that the producer gas by my process is not only purified of its nitrogen but it is also enriched 95 by a substantial addition of carbon monoxid, causing it to become a valuable by-product.

In carrying out the process in order to avoid a serious retardation of the reaction it is desirable to maintain such a flow of nitrogen through the furnace that the partial pressure of the carbon monoxid gas present will not exceed say 350 to 400 millimeters of mercury. The volatile carbo-nitrid thus produced may be recovered by leading it 100 from the furnace and allowing it to solidify or condense in suitable chambers, or by absorption in water or other solutions. If re-

covered by condensation, the solid thus obtained may be subjected to the action of water in a suitably closed vessel at substantially 200° C., when the following reaction takes place:—



- If the carbo-nitrid is recovered as a solution, the combined nitrogen may be converted into ammonia by heating the solution to substantially 200° C. in a suitably closed vessel. If the volatile product is allowed to condense as a loose powder when recovering it, it is apt to absorb any moisture with which it might come in contact and also to rapidly oxidize if exposed to free oxygen, and therefore care should be taken to prevent the exposure of this new product to water vapor or to the atmosphere.
- 20 In actual tests using magnesium oxid, carbon and nitrogen gas and a temperature of 1500° C. for 30 minutes analyses show that over 80% of the magnesium present in the magnesium oxid carried by the charge appeared in the volatile carbo-nitrid produced. These analyses further show chemically combined nitrogen as well as chemically combined carbon in the volatilized products in the proportion required by the formula 30  $\text{Mg}_3\text{N}_2\text{C}_3\text{N}_4$ . It is therefore certain that my volatile product is a carbo-nitrid and not a nitrid. The solid portion of the carbo-nitrid which is formed simultaneously with the volatile portion remains in the residue 35 passing through the furnace and its combined nitrogen may be recovered in the form of ammonia by treating said residue with water at about 200° C. in a suitably closed vessel.
- 40 The reactions of my new volatile product when hydrolyzed leads to the supposition that it produces a polymer of cyanamid in that it gives some of the characteristic reaction of melamin, such as a white precipitate with soluble silver and lead salts.

It is obvious that those skilled in the art may vary the details of my process without departing from the spirit of my invention, and therefore I do not wish to be limited to 50 the above disclosure except as may be required by the claims.

What I claim is:—

1. The process of producing a volatile magnesium carbo-nitrid, which consists in 55 preparing a mixture of magnesium oxid and carbon; and subjecting said mixture in an atmosphere containing free nitrogen to a

temperature sufficient to produce said volatile carbo-nitrid, substantially as described.

2. The process of producing a volatile 60 magnesium carbo-nitrid which consists in preparing a mixture of magnesium oxid and carbon; subjecting said mixture in an atmosphere containing nitrogen to a temperature sufficient to produce said carbo-nitrid, 65 and recovering the latter in a medium devoid of chemically active oxygen, substantially as described.

3. The process of producing a volatile 70 magnesium carbo-nitrid which consists in preparing a mixture of magnesium oxid and carbon; subjecting said mixture in an atmosphere of producer gas to a temperature sufficient to produce said carbo-nitrid, and recovering the latter in a medium devoid of 75 chemically active oxygen, substantially as described.

4. The process of producing a volatile magnesium carbo-nitrid, which consists in 80 preparing a mixture of magnesium oxid and carbon; and subjecting the same in an atmosphere containing nitrogen to a temperature sufficient to produce said carbo-nitrid thereby causing carbon-monoxid to be evolved while maintaining the partial pressure 85 of the carbon monoxid present below 400 millimeters of mercury, substantially as described.

5. The herein described new product containing chemically combined carbon nitrogen and magnesium the same being volatile 90 at 1500° C., capable of forming a soluble white powder and of producing a white precipitate with soluble silver and lead salts, as well as producing ammonia when subjected to the action of hot water, substantially as described.

6. The process of fixing nitrogen and simultaneously enriching producer gas which 100 consists in providing a mixture of magnesium oxid and carbon; feeding producer gas containing nitrogen thereto; and raising the temperature of said mixture sufficiently to cause some of said nitrogen to be removed from said gas by combining with magnesium 105 and carbon while also causing the carbon monoxid evolved to be added to the said producer gas, substantially as described.

In testimony whereof I affix my signature, in presence of two witnesses.

SAMUEL PEACOCK.

Witnesses:

T. A. WITHERSPOON,  
FRANCES SIEBEL.